

1

2,819,503

## METHOD OF PRODUCING RIMMED AND CAPPED STEEL

Vincent C. Boucek, Pittsburgh, Pa., assignor to United States Steel Corporation, a corporation of New Jersey

No Drawing. Application May 3, 1954  
Serial No. 427,346

5 Claims. (Cl. 22—215)

This invention relates generally to the manufacture of steel and, in particular, to the treatment of rimming steel after it has been teemed into ingot molds and before it has completely solidified therein.

This is a continuation-in-part of my application Serial No. 296,493, filed June 30, 1952, now abandoned.

For well known reasons, rimmed steel is desirable for certain products. Rimmed steel ingots as ordinarily produced, however, exhibit numerous blowholes adjacent the rim and segregation at the center in the upper portion thereof and such portion must accordingly be diverted to the manufacture of common products. Ingots made by the conventional practice including ladle and mold deoxidation, the use of rimming agents and a metal cap on the mold, furthermore, show excessive variation in case thickness and degree of center segregation, not only between ingots of different heats but even between ingots of the same heat. This introduces complications into the subsequent processing and working of the steel.

Attempts have been made heretofore to improve the quality of rimmed steel ingots. One of these, known as "chemical capping," is disclosed in Devaney Patent No. 2,108,254. The procedure there described includes the addition of sufficient deoxidizer after a predetermined period of rimming, to stop all rimming action in the ingot core or, in other words, to "kill" it. This practice, however, frequently produces ingots having dry or wet pipe which increases the amount of metal which must be scrapped.

It is accordingly the object of my invention to provide an improved method of treating rimming steel in the ingot mold so as to control more accurately the case thickness and to reduce the degree of center segregation in the top, thereby reducing the proportion of the ingot which must be diverted to common products.

From the standpoint of its action in the ingot mold, steel may be killed, semi-killed or rimming and the qualities and characteristics of each type are well understood. My invention concerns rimming steel only. According to the invention, speaking generally, I permit normal rimming of the ingot to occur for a predetermined time only. Then I add a deoxidizer to the core, i. e., the metal remaining molten in the upper central portion of the partially solidified ingot, to cause a gradual but incomplete deoxidation of the core. The amount of deoxidizer added should be sufficient to substantially arrest the rimming action but not sufficient either to cause crusting over or solidification of the top of the ingot or to prevent a continued rise of the metal in the top of the mold. I then apply a cap to the mold, whereupon the metal con-

2

tinues to rise in the top of the mold until it comes in contact with the cap, as in the case of a conventional capped ingot.

More specifically, in practicing the invention, I make a heat of rimming steel in the known manner, and partially deoxidize it in the ladle by the addition of ferromanganese, ferro-titanium, silico-manganese or aluminum or combinations thereof. The molten metal is then teemed into ingot molds as usual with the addition of known rimming agents and additional deoxidizers to obtain the amount of rimming action desired. The amount of rimming agent or deoxidizer needed for any ingot is adjusted by observing the rimming action of the ingots previously teemed from the same heat. According to conventional practice, the rimming of the ingots is allowed to proceed without check until the ingot has solidified. Alternatively, the rimming of capped steels is terminated after a few minutes, by placing a metal cap on top of the mold.

According to my invention, I permit rimming to proceed unrestrained for a predetermined period only, running from 1 minute to 10 or 12 minutes. This causes the formation of a case of solid metal of controlled thickness surrounding the still molten upper central portion or core. The longer the time, the thicker the case. After the desired rimming has occurred, I add a quantity of a deoxidizer in an amount sufficient to substantially arrest rimming and cause gradual but incomplete deoxidation without causing a crust to form on top of the metal or preventing further rise of the metal in the top of the mold. In other words, the amount of deoxidizer added should not exceed that which permits the ingot to remain open at the top. By such addition, the strong rimming action is reduced to a slow gentle movement on the surface of the metal. The deoxidizer should preferably be in comminuted form, i. e., small lumps or shot, and should be added slowly over an interval of time such as from 15 seconds to 40 or 50 seconds, to prevent excessive deoxidation localized in the core and resulting in a sharp demarcation between the case and core.

The deoxidizer which I prefer to employ is a commercially available calcium-silicon alloy containing 30 to 33% calcium, 60 to 60% silicon and the balance substantially iron. I may, however, use aluminum, ferrosilicon or the aluminum-silicon-iron alloy sold under the trade-mark "Alsifer."

The amount of deoxidizer to be added and the rate of addition can be determined by observation. The surface of the molten metal should exhibit a continuing rise during the addition. In other words, the rate and amount of addition should be controlled so as not to arrest the continuing rise which marks the proper degree of deoxidation. The amount of deoxidizer needed can also be checked by the appearance of macro-sections through billets rolled from the ingot. Such sections will be substantially free of oxides and pipe and if any blowholes are present they will be few and deep within the section if the proper amount of deoxidizer has been added. Too much deoxidizer gives evidence of pipe. Too little permits oxide segregation to persist in the core.

As soon as the addition of deoxidizer has been completed, a conventional metal mold cap is secured in position on top of the mold. The surface of the molten metal will continue to rise after placement of the cap and the

resulting elevation of the surface will bring it into contact with the cap as in the ordinary case of a capped ingot, as solidification proceeds inwardly to the center of the ingot. To insure this result, of course, the mold must be teemed to the proper level which can easily be determined by observing the action of the first few molds, and making any necessary correction as the teeming of the remaining molds proceeds. Ordinarily, the desired result will follow, in bottle top molds, if the mold be teemed to the level in the neck such that, after the predetermined period allowed for rimming, the molten metal will stand a safe distance, e. g., one inch, below the bottom of the cap when placed.

The time allowed for rimming and the amount of deoxidizer added thereafter just before capping, will depend, among other things, on the type of mold used, the size of the ingot and the particular grade of steel being made. The following table gives the significant data for typical examples of the method, using aluminum as the deoxidizer applied to ordinary steels of varying carbon content. In all the examples, ingots weighing approximately 9,000 lbs. were teemed into big-end-down bottle-top molds.

TABLE I

| Percent Carbon | Amount of Aluminum Added (Oz.) | Rimming Time (Min.) |
|----------------|--------------------------------|---------------------|
| .05            | 18                             | 8.5                 |
| .06-07         | 18                             | 6.5                 |
| .08-09         | 16                             | 4.5                 |
| .10-11         | 14                             | 4.5                 |
| .12 and over   | 14                             | 3                   |

In each case, the deoxidizer was added in the form of shot, about 3 oz. at a time, the addition extending over a period of from 15 to 40 seconds. The molds were teemed to such a level and the rimming was so controlled (by adding a rimming agent or a deoxidizer, as necessary) that the molten metal rose to within three inches of the top of the mold before the addition of the deoxidizer after the desired rimming. After addition of the deoxidizer, a metal cap was immediately placed on top of the mold.

As previously explained, the amount of deoxidizer added in each case must be carefully controlled so that it is sufficient to arrest the rimming action or nearly so but not sufficient to prevent a slight rise of the top of the ingot thereafter. With the proper amount of deoxidizer added, the steel rises and strikes the cap in about a minute. If an excess of deoxidizer be used, it causes the formation of pipe; if too little, oxide segregation will persist at the center. By "an excess of deoxidizer" I mean an amount in the range disclosed in the Devaney patent, such as .75 lb. of aluminum per ton of steel. Even an excess of 1 oz. of deoxidizer per ton, above the optimum amount, will cause some evidence of pipe. Using aluminum as the deoxidizer, ordinarily an amount of from 2.5 to 5 oz. per ton of ingot weight will suffice, i. e., amounts approximately one-third the minimum specified in the Devaney patent. In using calcium-silicon as the deoxidizer, somewhat larger amounts will be needed, i. e., as much as 8 oz. per ton of steel, but some advantage will be obtained by using an amount as small as 1 oz. per ton. The usual amount for an ingot of 4.5 tons is from 3 to 6 oz. per ton. If the aluminum or other deoxidizer be added all at once, instead of in steps or stages, a sharp demarcation between core and case results and pipe may form at the top of the ingot with oxide segregation persisting lower down.

When the ingot has solidified sufficiently, the cap is removed from the mold, the mold is stripped from the ingot and the ingot is subjected to soaking and working in the usual manner.

The chief advantage in my improved ingot practice is the fact that a large portion of oxygen in solution in

the liquid core of the ingot is fixed as a solid oxide most of which is fluxed off into the scum at the top of the ingot during the final gradual deoxidation. Comparatively few blowholes remain under the skin of the ingot, and the ingots can therefore be heated faster with the danger of burning the steel greatly reduced. Further, since there is much less gas pressure under the skin, it is not ruptured in rolling even though the skin may be very thin, and the billet surface obtained is much more nearly free of seams and slivers.

The invention is characterized by several other advantages, some of which have been mentioned briefly. In the first place, the thickness of case and degree of center segregation may be maintained substantially uniform not only throughout the same heat but also in separate heats. In addition, fully rimmed as well as thin-skinned capped steels can be produced by my method with improved results. The ingots are relatively free of oxide and sulphur segregation and pipe and the case thickness does not exceed a predetermined value. Under normal conditions, the cases are solid and uniform in depth from ingot to ingot. There is a minimum of segregation in the top of the ingots. As a result of these characteristics, it is no longer necessary to divert as large a percentage of the ingot to common products as heretofore. Finally, the segregation of carbon, phosphorus, manganese and sulphur across the section of the ingot is greatly reduced. This is shown by Table II giving the comparative billet re-check analysis for two ingots made by my invention (numbered 1 and 2) and a third ingot made by the conventional practice of capping shortly after teeming, for the purpose of comparison.

TABLE II

35. Comparative billet recheck analysis of mechanically and aluminum mechanically capped ingots, cross sectional sawings and section center drillings

|     | Percent Line | Sample | C   | Mn  | P    | S    | Total Al |
|-----|--------------|--------|-----|-----|------|------|----------|
| 40  | 7            | Ladle  | .12 | .54 | .095 | .057 | .007     |
|     | 7            | Saw    | .12 | .58 | .106 | .076 | .015     |
|     | 12           | Center | .14 | .59 | .136 | .102 | .015     |
|     | 12           | Saw    | .12 | .57 | .103 | .071 | .009     |
|     | 17           | Center | .13 | .57 | .114 | .083 | .015     |
|     | 17           | Saw    | .12 | .56 | .103 | .070 | .010     |
|     | 22           | Center | .11 | .56 | .097 | .064 | .012     |
|     | 22           | Saw    | .11 | .56 | .102 | .068 | .013     |
|     | 85           | Center | .08 | .54 | .090 | .051 | .005     |
|     | 85           | Saw    | .08 | .54 | .093 | .053 | .006     |
| 45  | 7            | Ladle  | .11 | .42 | .023 | .023 | .023     |
|     | 7            | Saw    | .10 | .46 | .013 | .027 | .027     |
|     | 12           | Center | .18 | —   | —    | .043 | .043     |
|     | 12           | Saw    | .10 | .46 | —    | .027 | .027     |
|     | 17           | Center | .18 | —   | —    | .044 | .044     |
|     | 17           | Saw    | .10 | .46 | —    | .027 | .027     |
|     | 22           | Center | .18 | —   | —    | .051 | .051     |
|     | 22           | Saw    | .10 | .46 | —    | .027 | .027     |
|     | 27           | Center | .16 | —   | —    | .037 | .037     |
|     | 27           | Saw    | .10 | .46 | —    | .027 | .027     |
| 50  | 62           | Center | .15 | .47 | —    | .036 | .036     |
|     | 62           | Saw    | .10 | .45 | —    | .025 | .025     |
|     | 92           | Center | .08 | .43 | —    | .028 | .028     |
|     | 92           | Saw    | .12 | .49 | .010 | .029 | .029     |
|     | 7            | Center | .15 | .53 | —    | .035 | .035     |
|     | 7            | Saw    | .31 | .59 | —    | .105 | .105     |
|     | 12           | Center | .14 | .53 | —    | .034 | .034     |
|     | 12           | Saw    | .28 | .58 | —    | .084 | .084     |
|     | 17           | Center | .14 | .53 | —    | .035 | .035     |
|     | 17           | Saw    | .31 | .58 | —    | .114 | .114     |
| 55  | 22           | Center | .20 | .54 | —    | .060 | .060     |
|     | 22           | Saw    | .13 | .52 | —    | .035 | .035     |
|     | 27           | Center | .19 | .53 | —    | .034 | .034     |
|     | 27           | Saw    | .13 | .52 | —    | .034 | .034     |
|     | 32           | Center | .17 | .53 | —    | .051 | .051     |
|     | 32           | Saw    | .13 | .52 | —    | .034 | .034     |
|     | 87           | Center | .12 | .52 | —    | .028 | .028     |
|     | 87           | Saw    | .10 | .50 | —    | .028 | .028     |
|     | 92           | Center | .12 | .50 | —    | .028 | .028     |
|     | 92           | Saw    | —   | —   | —    | —    | —        |
| 60  | 7            | Center | .31 | .59 | —    | .105 | .105     |
|     | 7            | Saw    | .14 | .53 | —    | .034 | .034     |
|     | 12           | Center | .28 | .58 | —    | .084 | .084     |
|     | 12           | Saw    | .14 | .53 | —    | .035 | .035     |
|     | 17           | Center | .31 | .58 | —    | .114 | .114     |
|     | 17           | Saw    | .13 | .52 | —    | .035 | .035     |
|     | 22           | Center | .20 | .54 | —    | .060 | .060     |
|     | 22           | Saw    | .13 | .52 | —    | .034 | .034     |
|     | 27           | Center | .19 | .53 | —    | .034 | .034     |
|     | 27           | Saw    | .13 | .52 | —    | .034 | .034     |
| 65  | 32           | Center | .17 | .53 | —    | .051 | .051     |
|     | 32           | Saw    | .13 | .52 | —    | .034 | .034     |
|     | 87           | Center | .12 | .52 | —    | .028 | .028     |
|     | 87           | Saw    | .10 | .50 | —    | .028 | .028     |
|     | 92           | Center | .12 | .50 | —    | .028 | .028     |
|     | 92           | Saw    | —   | —   | —    | —    | —        |
|     | 7            | Center | .31 | .59 | —    | .105 | .105     |
|     | 7            | Saw    | .14 | .53 | —    | .034 | .034     |
|     | 12           | Center | .28 | .58 | —    | .084 | .084     |
|     | 12           | Saw    | .14 | .53 | —    | .035 | .035     |
| 70  | 7            | Center | .31 | .59 | —    | .105 | .105     |
|     | 7            | Saw    | .14 | .53 | —    | .034 | .034     |
|     | 12           | Center | .28 | .58 | —    | .084 | .084     |
|     | 12           | Saw    | .14 | .53 | —    | .035 | .035     |
|     | 17           | Center | .31 | .58 | —    | .114 | .114     |
|     | 17           | Saw    | .13 | .52 | —    | .035 | .035     |
|     | 22           | Center | .20 | .54 | —    | .060 | .060     |
|     | 22           | Saw    | .13 | .52 | —    | .034 | .034     |
|     | 27           | Center | .19 | .53 | —    | .034 | .034     |
|     | 27           | Saw    | .13 | .52 | —    | .034 | .034     |
| 75  | 32           | Center | .17 | .53 | —    | .051 | .051     |
|     | 32           | Saw    | .13 | .52 | —    | .034 | .034     |
|     | 87           | Center | .12 | .52 | —    | .028 | .028     |
|     | 87           | Saw    | .10 | .50 | —    | .028 | .028     |
|     | 92           | Center | .12 | .50 | —    | .028 | .028     |
|     | 92           | Saw    | —   | —   | —    | —    | —        |
|     | 7            | Center | .31 | .59 | —    | .105 | .105     |
|     | 7            | Saw    | .14 | .53 | —    | .034 | .034     |
|     | 12           | Center | .28 | .58 | —    | .084 | .084     |
|     | 12           | Saw    | .14 | .53 | —    | .035 | .035     |
| 80  | 7            | Center | .31 | .59 | —    | .105 | .105     |
|     | 7            | Saw    | .14 | .53 | —    | .034 | .034     |
|     | 12           | Center | .28 | .58 | —    | .084 | .084     |
|     | 12           | Saw    | .14 | .53 | —    | .035 | .035     |
|     | 17           | Center | .31 | .58 | —    | .114 | .114     |
|     | 17           | Saw    | .13 | .52 | —    | .035 | .035     |
|     | 22           | Center | .20 | .54 | —    | .060 | .060     |
|     | 22           | Saw    | .13 | .52 | —    | .034 | .034     |
|     | 27           | Center | .19 | .53 | —    | .034 | .034     |
|     | 27           | Saw    | .13 | .52 | —    | .034 | .034     |
| 85  | 32           | Center | .17 | .53 | —    | .051 | .051     |
|     | 32           | Saw    | .13 | .52 | —    | .034 | .034     |
|     | 87           | Center | .12 | .52 | —    | .028 | .028     |
|     | 87           | Saw    | .10 | .50 | —    | .028 | .028     |
|     | 92           | Center | .12 | .50 | —    | .028 | .028     |
|     | 92           | Saw    | —   | —   | —    | —    | —        |
|     | 7            | Center | .31 | .59 | —    | .105 | .105     |
|     | 7            | Saw    | .14 | .53 | —    | .034 | .034     |
|     | 12           | Center | .28 | .58 | —    | .084 | .084     |
|     | 12           | Saw    | .14 | .53 | —    | .035 | .035     |
| 90  | 7            | Center | .31 | .59 | —    | .105 | .105     |
|     | 7            | Saw    | .14 | .53 | —    | .034 | .034     |
|     | 12           | Center | .28 | .58 | —    | .084 | .084     |
|     | 12           | Saw    | .14 | .53 | —    | .035 | .035     |
|     | 17           | Center | .31 | .58 | —    | .114 | .114     |
|     | 17           | Saw    | .13 | .52 | —    | .035 | .035     |
|     | 22           | Center | .20 | .54 | —    | .060 | .060     |
|     | 22           | Saw    | .13 | .52 | —    | .034 | .034     |
|     | 27           | Center | .19 | .53 | —    | .034 | .034     |
|     | 27           | Saw    | .13 | .52 | —    | .034 | .034     |
| 95  | 32           | Center | .17 | .53 | —    | .051 | .051     |
|     | 32           | Saw    | .13 | .52 | —    | .034 | .034     |
|     | 87           | Center | .12 | .52 | —    | .028 | .028     |
|     | 87           | Saw    | .10 | .50 | —    | .028 | .028     |
|     | 92           | Center | .12 | .50 | —    | .028 | .028     |
|     | 92           | Saw    | —   | —   | —    | —    | —        |
|     | 7            | Center | .31 | .59 | —    | .105 | .105     |
|     | 7            | Saw    | .14 | .53 | —    | .034 | .034     |
|     | 12           | Center | .28 | .58 | —    | .084 | .084     |
|     | 12           | Saw    | .14 | .53 | —    | .035 | .035     |
| 100 | 7            | Center | .31 | .59 | —    | .105 | .105     |
|     | 7            | Saw    | .14 | .53 | —    | .034 | .034     |
|     | 12           | Center | .28 | .58 | —    | .084 | .084     |
|     | 12           | Saw    | .14 | .53 | —    | .035 | .035     |
|     | 17           | Center | .31 | .58 | —    | .114 | .114     |
|     | 17           | Saw    | .13 | .52 | —    | .035 | .035     |
|     | 22           | Center | .20 | .54 | —    | .060 | .060     |
|     | 22           | Saw    | .13 | .52 | —    | .034 | .034     |
|     | 27           | Center | .19 | .53 | —    | .034 | .034     |
|     | 27           | Saw    | .13 | .52 | —    | .034 | .034     |
| 105 | 32           | Center | .17 | .53 | —    | .051 | .051     |
|     | 32           | Saw    | .13 | .52 | —    | .034 | .034     |
|     | 87           | Center | .12 | .52 | —    | .028 | .028     |
|     | 87           | Saw    | .10 | .50 | —    | .028 | .028     |
|     | 92           | Center | .12 | .50 | —    | .028 | .028     |
|     | 92           | Saw    | —   | —   | —    | —    | —        |
|     | 7            | Center | .31 | .59 | —    | .105 | .105     |
|     | 7            | Saw    | .14 | .53 | —    | .034 | .034     |
|     | 12           | Center | .28 | .58 | —    | .084 | .084     |
|     | 12           | Saw    | .14 | .53 | —    | .035 | .035     |
| 110 | 7            | Center | .31 | .59 | —    | .105 | .105     |
|     | 7            | Saw    | .14 | .53 | —    | .034 | .034     |
|     | 12           | Center | .28 | .58 | —    | .084 | .084     |
|     | 12           | Saw    | .14 | .53 | —    | .035 | .035     |
|     | 17           | Center | .31 | .58 | —    | .114 | .114     |
|     | 17           | Saw    | .13 | .52 | —    | .035 | .035     |
|     | 22           | Center | .   |     |      |      |          |

TABLE III  
*Calcium silicon precapped ingots*

| Ingot Number | 16        |           | 20                |           | 24                |           |
|--------------|-----------|-----------|-------------------|-----------|-------------------|-----------|
|              | Sawings   |           | 1/4" Center Drill |           | 1/4" Center Drill |           |
| Type Sample  | Percent C | Percent S | Percent C         | Percent S | Percent C         | Percent S |
|              | Percent C | Percent S | Percent C         | Percent S | Percent C         | Percent S |
| 7            | .14       | .021      | .15               | .017      | .12               | .017      |
| 12           | .17       | .027      | .20               | .030      | .12               | .021      |
| 17           | .15       | .029      | .23               | .044      | .21               | .034      |
| 22           | .16       | .028      | .19               | .034      | .18               | .034      |
| 27           | .16       | .029      | .17               | .033      | .18               | .032      |
| 32           | .16       | .027      | .16               | .031      | .20               | .037      |
| 42           | .14       | .026      | .16               | .027      |                   |           |
| 52           | .13       | .026      | .15               | .027      |                   |           |
| 62           | .14       | .025      | .14               | .026      |                   |           |
| 72           | .14       | .025      | .14               | .025      |                   |           |
| 82           | .13       | .025      | .12               | .023      |                   |           |
| 92           | .12       | .022      | .13               | .023      |                   |           |
| Rimming Time | 3 Minutes |           | 3 Minutes         |           | 3 Minutes         |           |

For the purpose of comparison, Table IV gives a similar showing taken from ingots made from the same heat by the conventional mechanical capping procedure.

TABLE IV  
*Mechanically capped ingots*

| Ingot Number | 2                 |           | 4                 |           | 8                 |           | 15        |                   |
|--------------|-------------------|-----------|-------------------|-----------|-------------------|-----------|-----------|-------------------|
|              | 1/4" Center Drill |           | 1/4" Center Drill |           | 1/4" Center Drill |           | Sawings   | 1/4" Center Drill |
| Type Sample  | Percent C         | Percent S | Percent C         | Percent S | Percent C         | Percent S | Percent C | Percent S         |
|              | Percent C         | Percent S | Percent C         | Percent S | Percent C         | Percent S | Percent C | Percent S         |
| 7            | .28               | .059      | .40               | .125      | .28               | .073      | .17       | .032              |
| 12           | .22               | .049      | .22               | .048      | .28               | .070      | .17       | .031              |
| 17           |                   |           |                   |           |                   |           | .16       | .028              |
| 22           | .18               | .032      | .19               | .043      | .19               | .050      | .17       | .028              |
| 27           |                   |           |                   |           |                   |           | .16       | .027              |
| 32           |                   |           |                   |           |                   |           | .16       | .021              |
| 42           |                   |           |                   |           |                   |           | .14       | .046              |
| 52           |                   |           |                   |           |                   |           | .15       | .026              |
| 62           |                   |           |                   |           |                   |           | .14       | .026              |
| 72           |                   |           |                   |           |                   |           | .13       | .029              |
| 82           |                   |           |                   |           |                   |           | .12       | .025              |
| 92           |                   |           |                   |           |                   |           | .13       | .025              |
| Rimming Time | 1 Minute          |           | 13 Minutes        |           | 2 Minutes         |           | 3 Minutes |                   |

For further comparison, Table V gives the results obtained in one ingot made from the same heat by adding an excess of 1 oz. per ton of calcium-silicon to the core after a rimming time of 3 minutes. Although segregation therein is less than in the ingots listed in Table IV, it was not as low as in the ingots listed in Table III. In addition, the small excess of deoxidizer caused a pipe to appear and the top portion of the ingot therefore had to be scrapped.

TABLE V  
*Calcium silicon capped—no mechanical cap*

| Ingot Number | 25                |           |
|--------------|-------------------|-----------|
|              | 1/4" Center Drill |           |
| Type Sample  | Percent Line      |           |
|              | Percent C         | Percent S |
| 7            |                   |           |
| 12           |                   |           |
| 17           |                   |           |
| 22           |                   |           |
| 27           |                   |           |
| Rimming Time | .19               | .041      |
|              | .19               | .052      |
|              | .20               | .049      |
|              | 3 Minutes         |           |

A comparison of the center drillings shows that there is no significant difference in segregation with either practice below the 32% line. With the mechanical capping

practice (ingots 2, 4, 8 and 15) segregation increases progressively to the top of the ingot. With the calcium silicon precap practice (ingots 16, 20 and 24) the segregation increases but at a much slower rate to the 17% line.

5 Above the 17% line to the top of ingot segregation decreases.

Of special significance is the fact that the maximum segregation on calcium-silicon precapped steel with no top diversion is less (.044% S—center drill #16 ingot 10 17% line) than on mechanically capped steel with a 20% top diversion (.050% S—#8 ingot 27% line).

The highest segregation on the calcium-silicon precapped steel analyzed only .23% C and .044% S (ingot 15 #16, 17% line center drill).

15 Chemical capping with 23 ounces of calcium silicon (#25 ingot) does not retard segregation as well as the combination of precapping with 18 ounces of calcium silicon and then mechanically capping. Further, a bad slag pipe was evident on the etch test of ingot #25 at the 20 7% line.

The improved quality of the ingots produced by my invention is shown by Table VI comparing the results obtained therefrom with those of the conventional capping practice.

25

TABLE VI  
*Ingot practice*

|                                             | Conventional Capping | Rimming, Deoxidation and capping as disclosed herein |
|---------------------------------------------|----------------------|------------------------------------------------------|
| Number of heats involved                    | 101                  | 99                                                   |
| Ingot yield of cold-heading quality percent | 53.1                 | 73                                                   |
| Billet diversion to common products percent | 32.2                 | 11.4                                                 |
| 60 Billet rejections:                       |                      |                                                      |
| Seabs, Pipe, Seams, Burns, Tears percent    | .52                  | .36                                                  |
| Mechanical defects and bent billets do      | .11                  | .09                                                  |
| Total do                                    | .63                  | .45                                                  |

65 A further advantage of the invention is that it reduces the necessary amount of hot-process deseaming of billets to be rolled in rod mills, thus materially decreasing cost as compared to prior practice.

Although I have disclosed herein the preferred embodiment and practice of my invention, I intend to cover as well any change or modification therein which may be made without departing from the spirit and scope of the invention.

I claim:

75 1. The method of producing rimmed steel ingots which

consists in teeming rimming steel into an ingot mold, allowing the steel in the mold to rim for from 1 to 12 minutes, progressively adding to the core of the ingot then remaining molten a deoxidizer in the amount of from 11 to 8 ounces per ton of ingot weight, over a period of from 15 to 50 seconds and then applying a metal cap to the mold.

2. The method defined by claim 1 characterized by said deoxidizer being calcium-silicon alloy.

3. The method defined by claim 1 characterized by 10 said deoxidizer being aluminum.

4. The method of producing rimmed steel ingots which consists in teeming rimming steel into an ingot mold, allowing the steel in the mold to rim for a few minutes, then while the steel is still effervescent, progressively adding to the core then remaining molten, over a period of from 15 to 50 seconds, sufficient deoxidizer to substantially arrest the rimming action but less than the amount needed to prevent a continued rise of metal in the mold, and then applying a metal cap to the mold.

5. The method of making rimmed steel which consists in teeming a heat of molten rimming steel into ingot molds, allowing the steel to stand in the molds for undisturbed rimming to produce the desired thickness of case, then, while the steel is still effervescent at the top of the mold, progressively arresting the rimming action by progressively adding to the central core of the steel mass remaining molten, a deoxidizer in an amount of

5 from 1 to 8 ounces per ton of ingot weight, thereby substantially arresting the rimming action of said core yet preventing excessive localized deoxidation in the core by causing the top of the core to remain open with continued rise to the metal, and thereby eliminating the sharp demarcation between case and core then placing a metal cap on top of the mold and, in conducting said teeming, filling the molds to a level such that said continued rise of the top of the core brings the teemed metal into contact with said cap.

References Cited in the file of this patent

UNITED STATES PATENTS

|    |           |                 |                |
|----|-----------|-----------------|----------------|
| 15 | 587,105   | McConnell       | July 27, 1897  |
|    | 1,727,088 | Williams et al. | Sept. 3, 1929  |
|    | 2,108,254 | Devaney         | Feb. 15, 1938  |
|    | 2,204,585 | Gagnebin        | June 18, 1940  |
|    | 2,652,324 | Hignett         | Sept. 15, 1953 |

20 OTHER REFERENCES

The Deoxidation of Steel, C. H. Herty, Bulletin No. 69, 1934, pages 41-42 relied on.

Open Hearth Proceedings, vol. 32, 1949, A. I. M. E., page 226.

25 Open Hearth Proceedings, vol. 34, 1951, A. I. M. E., pages 234-237.

The Making, Shaping, and Treating of Steel, U. S. Steel (6th ed.) 1951, pages 444, 571-573 relied on.

U. S. DEPARTMENT OF COMMERCE  
PATENT OFFICE  
CERTIFICATE OF CORRECTION

January 14, 1958

Patent No. 2,819,503

Vincent C. Boucek

It is hereby certified that error appears in the printed specification of the above numbered patent requiring correction and that the said Letters Patent should read as corrected below.

Column 2, line 44, for "60 to 60%" read -- 60 to 65% --; column 8, line 5, for "rise to" read -- rise of --.

Signed and sealed this 11th day of March 1958.

(SEAL)

Attest:

KARL H. AXLINE

Attesting Officer

ROBERT C. WATSON  
Commissioner of Patents